

# United States Patent [19]

Hildebrand et al.

[11] 3,785,767

[45] Jan. 15, 1974

[54] **PROCESS FOR THE CONTINUOUS DYEING AND PRINTING OF FIBRE MATERIALS CONTAINING IONIC GROUPS**

[75] Inventors: Dietrich Hildebrand, Odenthal; Robert Kuth, Cologne, both of Germany

[73] Assignee: **Bayer Aktiengesellschaft**, Leverkusen, Germany

[22] Filed: **Aug. 10, 1970**

[21] Appl. No.: **62,651**

[30] **Foreign Application Priority Data**

Aug. 16, 1969 Germany ..... 1941698

[52] **U.S. Cl.** ..... **8/54**, 8/94, 8/168, 8/174, 8/169

[51] **Int. Cl.** ..... **D06p 3/14**

[58] **Field of Search** ..... 8/94, 168, 174, 173, 8/178, 6, 54

[56] **References Cited**

UNITED STATES PATENTS

|           |         |                |        |
|-----------|---------|----------------|--------|
| 3,510,243 | 5/1970  | Seuret et al.  | 8/94 X |
| 2,721,111 | 10/1955 | Long et al.    | 8/6 X  |
| 3,164,449 | 1/1965  | Buxbaum        | 8/6 X  |
| 2,274,751 | 3/1942  | Sowter et al.  | 8/173  |
| 3,523,749 | 8/1970  | MacLeod et al. | 8/54.2 |

3,623,834 11/1971 Seuret et al. .... 8/173

FOREIGN PATENTS OR APPLICATIONS

|           |        |             |         |
|-----------|--------|-------------|---------|
| 682,830   | 1/1966 | Belgium     | 8/174   |
| 454,084   | 6/1968 | Switzerland | 8/178 R |
| 1,581,325 | 8/1969 | France      | 8/94    |

OTHER PUBLICATIONS

Colour Index, 2nd Ed., 1956, Vol. 2, pp. 2815 and 2816.

Primary Examiner—Donald Levy

Assistant Examiner—T. J. Herbert, Jr.

Attorney—Plumley and Tyner

[57]

ABSTRACT

Pad-steaming process for the continuous dyeing and printing of fibre materials containing ionic groups, from organic solvents, characterised in that the fibre materials are dyed or printed with chlorinated hydrocarbon dyeing baths containing ionic dyestuffs which have been rendered soluble in chlorinated hydrocarbons by the formation of salts or addition products with lipophilic compounds.

With the new process, it is possible to produce on fibre materials containing ionic groups strong, level and well developed dyeings and prints in excellent yields.

8 Claims, No Drawings

**PROCESS FOR THE CONTINUOUS DYEING AND PRINTING OF FIBRE MATERIALS CONTAINING IONIC GROUPS**

The invention relates to a pad-steaming process for the continuous dyeing and printing of fibre materials containing ionic groups, from organic solvents; the process is characterised in that the fibre materials are dyed or printed with chlorinated hydrocarbon dyebaths containing ionic dyestuffs which have been rendered soluble in chlorinated hydrocarbons by the formation of salts or addition products with lipophilic compounds.

Chlorinated hydrocarbons suitable for the process according to the invention are primarily the chlorinated hydrocarbons the boiling points of which lie between 40° and 170°C, e.g. aliphatic chlorinated hydrocarbons such as methylene chloride, chloroform, carbon tetrachloride, 1,1-dichloroethane, 1,2-dichloroethane, 1,1,1-trichloroethane, 1,1,2-trichloroethane, 1,1,1,2-tetrachloroethane, 1,1,2,2-tetrachloroethane, pentachloroethane, 1-chloropropane, 1,2-dichloropropane, 1-chlorobutane, 2-chlorobutane, 1,4-dichlorobutane, 1-chloro-2-methylpropane, 2-chloro-2-methylpropane or 4-chloro-2-methylpropane, and aromatic chlorinated hydrocarbons such as chlorobenzene and chlorotoluene. Tetrachloroethylene, trichloroethylene and 1,1-trichloropropane have proved particularly satisfactory.

The fibre materials containing ionic groups, which are to be dyed according to the invention comprise:

a. fibre materials containing cationic groups.

These include all natural or synthetic fibre materials which can be dyed with anionic dyestuffs. These are natural polyamides especially wool and synthetic polyamides, e.g., poly- $\epsilon$ -caprolactam, polyhexamethylene-diamine adipate and poly- $\omega$ -amino-undecanic acid;

b. fibre materials containing anionic groups.

These include all synthetic fibre materials which can be dyed with basic dyestuffs, especially the commercial polyacrylonitrile containing anionic groups such as sulphonate acid, sulphimide, carboxyl and/or phosphonic acid groups; polyesters modified by carboxyl and/or sulphonate acid groups, such as polyethylene terephthalate, polycyclohexane-dimethylene terephthalate; heterogeneous polyesters obtained from terephthalic acid, isophthalic acid and ethylene glycol or from terephthalic acid, sulphoisophthalic acid and ethylene glycol; furthermore, copolyether ester fibres obtained from p-hydroxybenzoic acid, terephthalic acid and ethylene glycol; or polyamides modified by sulphonate acid groups, such as polyhexamethylene adipate, polycaprolactam of poly- $\omega$ -aminoundecanic acid.

The ionic dyestuffs which have been rendered soluble in chlorinated hydrocarbons by the formation of salts or addition products with lipophilic compensating ions and serve in the process according to the invention for the dyeing of fibre materials containing cationic groups comprise chlorinated hydrocarbon-soluble amine salts and amine addition products of dyestuffs containing 1 to 4 carboxyl and/or sulphonate acid groups.

The dyestuffs containing 1 to 4 sulphonate acid groups from which the amine salts or amine addition products soluble in chlorinated hydrocarbons are derived, may belong to a variety of dyestuff classes, for example, to

the azo, anthraquinone, phthalocyanine, azine and triphenyl-methane dyestuffs. These dyestuffs may also contain reactive groups.

Suitable amines on which the amine salts or amine addition products soluble in chlorinated hydrocarbons are based, are primary, secondary and tertiary monoamines as well as primary, secondary and tertiary polyamines. Examples of primary, secondary and tertiary monoamines are:

- 10 optionally substituted aliphatic amines, such as tri-n-propylamine, 2-ethyl-hexylamine, dodecylamine, dodecylamine polyglycol ether with 20 mol ethylene oxide, hexadecylamine, hexadecylamine polyglycol ether with 20 mol ethylene oxide, octadecylamine, N-methyl-octadecylamine, 15 N-methyl-octadecylamine polyglycol ether with 10 mol ethylene oxide, cetylamine, N,N-dimethyl-dodecylamine, N,N-dimethyl-hexadecylamine, N,N-dimethyl-octadecylamine, 20 N,N-dibutyl-dodecylamine, N,N-di-2-hydroxyethyl-oleylamine, N,N-dimethyl-N-(dodecanoylaminomethyl)-amine, N-methyl-N-2-hydroxyethyl-N-[ $\gamma$ -octadecanoylamino]-propyl]-amine,  $\epsilon$ -aminocapronic acid butyl ester,  $\epsilon$ -aminocapronic acid dodecylamide,  $\epsilon$ -aminoundecanic acid butyl ester; technical mixtures of 25 fatty amines, such as coconut fatty amine and sperm oil fatty amines and their ethoxylation and propoxylation products; optionally substituted cycloaliphatic amines, such as N,N-dimethyl-cyclohexylamine, 30 N-ethyl-cyclohexylamine, N-2-hydroxyethyl-cyclohexylamine, N,N-bis-(2-hydroxyethyl)-cyclohexylamine, N,N-bis-(2-chloroethyl)-cyclohexylamine, 35 1-cyclohexylamino-propanol-2, 1-cyclohexylamino-propylamine-3 and dicyclohexylamine; optionally substituted araliphatic amines, such as benzylamine, N,N-dimethyl-benzylamine, 40 N,N-dibenzylamine, N-methyl-N,N-dibenzylamine, 45 1-amino-1-phenyl-ethane, 1-amino-2-ethane; optionally substituted aromatic amines, such as N-ethyl-aniline, 50 N,N-dimethyl-aniline, N,N-diethyl-aniline, N-propyl-aniline, N,N-dipropyl-aniline, 55 N-butyl-aniline, N-isobutyl-aniline, N-(2-chloroethyl)-N-butyl-aniline, N-2-hydroxyethyl-aniline, N-methyl-N-(2-hydroxyethyl)-aniline, 60 N-butyl-N-(2-hydroxyethyl)-aniline, N,N-bis-(2-hydroxyethyl)-aniline, N-methyl-N-(2-cyanoethyl)-aniline,

2-amino-toluene,  
 2-methylamino-toluene,  
 2-dimethylamino-toluene,  
 2-ethylamino-toluene,  
 3-amino-toluene,  
 3-dimethylamino-toluene,  
 3-ethylamino-toluene,  
 3-butylamino-toluene,  
 3(N-ethyl-N-hydroxyethyl)-amino-toluene,  
 3-[N-bis-(2-hydroxyethyl)]-amino-toluene,  
 3-[N-ethyl-N-(2-dimethylaminoethyl)]-amino-toluene,  
 4-methylamino-toluene,  
 4-dimethylamino-toluene,  
 4-ethylamino-toluene,  
 4-diethylamino-toluene,  
 N-ethyl-N-benzyl-aniline,  
 3-(N-ethyl-N-benzyl)-amino-toluene,  
 xylidine,  
 2-iso-propyl-aniline,  
 2-methyl-6-ethyl-aniline,  
 2,6-diisopropyl-aniline,  
 4-dodecyl-aniline,  
 N,N-dimethyl-4-dodecyl-aniline,  
 5,6,7,8-tetrahydro-naphthylamine-(1),  
 1-diethylamino-naphthalene,  
 4,4'-diamino-dicyclohexylmethane,  
 optionally substituted heterocyclic amines, such as  
 N-propyl-morpholine,  
 N-hexyl-morpholine,  
 N-dodecyl-morpholine,  
 N-hexadecyl-morpholine,  
 N-dodecyl-piperidine,  
 N-hexadecyl-piperidine,  
 N-dodecyl-imidazole,  
 2-dodecyl-hydroindole,  
 N-dodecyl-benzimidazole,  
 2-dodecyl-benzimidazole,  
 1-( $\beta$ -hydroxyethyl)2-octadecyl-imidazoline,  
 1-( $\beta$ -octadecanoylaminoethyl)2-octadecyl-  
 imidazoline.

Examples of primary, secondary and tertiary polyamines are primarily aliphatic polyamines, such as  
 N-dodecyl-N',N'-dimethyl-ethylene-diamine,  
 N-dodecyl-N',N'-diethyl-ethylene-diamine,  
 N-octadecyl-N',N'-diethyl-ethylene-diamine,  
 N-phenyl-N',N'-dimethyl-ethylene-diamine,  
 N-oleyl-N',N'-dimethyl-ethylene-diamine,  
 N-oleyl-N',N'-diethyl-ethylene-diamine,  
 N-dodecyl-N',N'-dimethyl-propylene-diamine-(1,3),  
 N-dodecyl-N',N'-diethyl-propylene-diamine-(1,3),  
 N-oleyl-N',N'-dimethyl-propylene-diamine-(1,3),  
 N-oleyl-N',N'-diethyl-propylene-diamine-(1,3),  
 N-dodecyl-ethylene-triamine,  
 N-dodecyl-ethylene-tetramine,  
 N-octadecyl-ethylene-tetramine.

If acidic dyestuffs containing reactive groups are used, obviously, only those amines are suitable for the formation of salts or addition products, which contain no free NH-group.

Ionic dyestuffs which have been rendered soluble in chlorinated hydrocarbons by the formation of salts or addition products with lipophilic compounds and serve in the process according to the invention for the dyeing of fibre materials containing anionic groups comprise all cationic dyestuffs which contain at least one cationic nitrogen atom and the anion of an acid which

forms a salt soluble in chlorinated hydrocarbons with the cationic dyestuff.

The cationic dyestuffs from which the dyestuff salts to be used according to the invention, which contain at least one cationic nitrogen atom and are soluble in chlorinated hydrocarbons are derived, may belong to a variety of dyestuff classes, for example, to the azo, anthraquinone, azine, oxazine, xanthene, methine, triphenyl-methane and phthalocyanine dyestuffs. The dyestuffs include optical brightening agents, e.g. optical brightening agents from the stilbene, coumarin, azole, and naphthalimide series.

Anions suitable for the dyestuff salts are:  
 anions of acidic esters of inorganic acids, such as the

15 dodecyl sulphate,  
 stearyl sulphate,  
 oleyl sulphate,  
 oleic acid sulphate,  
 oleic acid butyl ester sulphate,  
 20 ricinoleic acid ethyl ester sulphate,  
 ricinoleic acid monoethyl glycol ester sulphate,  
 oleic acid ethylamide sulphate,  
 oleic acid ethanolamide sulphate,  
 oleic acid diethanolamide sulphate,  
 25 oleic acid diisobutylamide sulphate,  
 oleic acid anilide sulphate,  
 N-acetyloleylamine sulphate,  
 undecylethylene glycol ether sulphate,  
 tetradecyltriglycol ether sulphate,  
 30 hexadecylglycol ether sulphate,  
 octadecylpentaglycol ether sulphate,  
 N-oleyl-4-aminobutano-2-sulphate ions and



40 anions of organic acids, such as  
 oleic acid-N-dimethylamide sulphonate,



45  $\text{C}_{12}\text{-C}_{17}$ -paraffin sulphonate,  
 n-butylbenzene sulphonate,  
 n-amylbenzene sulphonate,  
 N-hexylbenzene sulphonate,  
 n-heptylbenzene sulphonate,  
 50 diisopropylnaphthalene sulphonate,  
 dibutylnaphthalene sulphonate,  
 di-(diisobutyl-methyl)-naphthalene sulphonate,  
 dibutylphenyl polyglycol ether sulphate,  
 n-octylbenzene sulphonate,  
 55 n-nonylbenzene sulphonate,  
 n-decylbenzene sulphonate,  
 n-dodecylbenzene sulphonate,  
 n-tetradecylbenzene sulphonate,  
 n-hexadecylbenzene sulphonate,  
 n-octadecylbenzene sulphonate,  
 60 2-ethyl-hexylbenzene sulphonate,  
 2-propyl-heptylbenzene sulphonate,  
 2-butyl-octylbenzene sulphonate,  
 2-amyl-nonylbenzene sulphonate,  
 65 dodecyl-(6)-benzene sulphonate and  
 tetrapropylene benzene sulphonate ions;  
 and also the

palmitate, stearate, oleate ions.

The amounts in which the dyestuff amine salts or addition products or the salts of dyestuff bases with aliphatic or aromatic carboxylic or sulphonic acids to be used according to the invention are added to the chlorinated hydrocarbon padding liquors may vary within wide limits, dependent upon the desired depth of colour; in general, amounts of 5 g to 30 g in 1000 g of padding liquor have proved satisfactory.

In the process according to the invention it has frequently proved useful, in order to increase the viscosity of the padding liquors, to add to the padding liquors about 8 to 10 per cent by weight of water, referred to the weight of the chlorinated hydrocarbons, and 0 to 5 per cent by weight, referred to the weight of the chlorinated hydrocarbons, of emulsifiers which form thickened emulsions with the chlorinated hydrocarbons when water is added. Suitable thickening emulsifiers are commercial non-ionic, anion-active, cation-active or zwitterionic emulsifiers, for example, oleic acid ethanolamide, oleyl alcohol eicosaglycol ether, nonylphenol heptaglycol ether, nonylphenol decaglycol ether, dodecylbenzene sulphonate, stearyl alcohol sulphate, N,N-dimethyl-N-benzyl-N-oleyl ammonium chloride and N,N-dimethyl-N-hexadecyl-N-(2-hydroxy-3-sulpho)-propylbataine.

Furthermore, the chlorinated hydrocarbon dyebaths may contain auxiliaries which further the fixing of the dyestuff and/or improve the quality of the dyeing, for example, the levelness. Auxiliaries which have proved satisfactory are, for example, interface-active compounds which are soluble in chlorinated hydrocarbons, such as alkylbenzene sulphonates, fatty alcohol sulphates, ethoxylation products of fatty alcohols, alkylphenols, fatty amines, fatty acid amides and fatty acids; furthermore, fatty acid ethanolamides, fatty amine oxides, fatty acid amideamine oxides, as well as mixtures thereof. The quantities in which the auxiliaries are added to the dyebath amount to 0 - 4%, preferably 0.5 - 2%, referred to the fibre material to be dyed. Furthermore, the dyebaths may contain 0.1 - 2 per cent by weight, referred to the weight of the chlorinated hydrocar-

in undissolved form. However, it has also proved satisfactory to add them to the chlorinated hydrocarbons in the form of concentrated, e.g., 25 - 50%, solutions in chlorinated hydrocarbons or in organic solvents of unlimited miscibility with the latter, such as dimethyl formamide, isopropanol, diethylene glycol monoethyl ether, diethylene glycol monobutyl ether, ethylene glycol monoisopropyl ether, ethylene glycol monobutyl ether, benzyl alcohol or butyrolactone.

From Swiss Patent Specification No. 454,084 there is known a process for the continuous dyeing of textile materials of synthetic polyamides from organic solvents, in which the textile materials are dyed or printed with dyebaths containing disperse dyestuffs or water-soluble dyestuffs in solvent mixtures. Compared with this process, the process according to the invention in which dyestuffs soluble in chlorinated hydrocarbons are used, is superior in that it yields stronger and more brilliant dyeing and prints, since the good solubility of the dyestuffs to be used according to the invention, in chlorinated hydrocarbons - even without the addition of solubilizers - enables stable single-phase padding liquors of high dyestuff concentrations to be prepared. Moreover, the use of dyestuffs soluble in chlorinated hydrocarbons according to the invention makes it possible to rinse the fibre materials with chlorinated hydrocarbons so that the whole dyeing process can be carried out without the occurrence of waste water.

With the aid of the process according to the invention it is possible to produce on fibre materials containing ionic groups strong, lever and well developed dyeings and prints of outstanding fastness properties in excellent yields and without the occurrence of waste water, while the original textile fibre properties of the dyed material are retained to the optimal extent.

The parts given in the following Examples are parts by weight.

#### EXAMPLE 1

A wool fabric is padded on a foulard with a thickened padding liquor consisting of  
20 parts of the dyestuff of the formula



bonds, of a lower carboxylic acid, such as formic acid or acetic acid.

The process according to the invention is advantageously carried out by spraying or impregnating the fibre materials with the chlorinated hydrocarbon liquors, squeezing to a liquor absorption of 60 - 160%, and then treating them, optionally after an intermediate drying, with saturated steam or overheated steam at 100° - 200°C. The fibre materials are subsequently rinsed with chlorinated hydrocarbons, in order to remove the non-fixed dyestuff, and subsequently dried by blowing with hot air.

The dyestuffs soluble in chlorinated hydrocarbons can be added to the chlorinated hydrocarbons liquors

55 2 parts nonylphenol decaglycol ether,  
898 parts perchloroethylene and  
80 parts of water  
60 with a liquor absorption of 105%, steamed at 102°C for  
10 minutes, subsequently rinsed three times with perchloroethylene at room temperature and dried by  
blowing with hot air.

Without the occurrence of waste water, there is obtained a wool fabric which is dyed in a level red shade and has a substantially better appearance than a fabric dyed in an aqueous solution.

#### EXAMPLE 2

A wool fabric is impregnated with a padding liquor

consisting of  
20 parts of the dyestuff of the formula



### 10 parts of a compound of the formula



6 parts 1,3-bis-(2-ethyl-hexyl)-glycerol ether sulphate,  
 2 parts isononyl phenol heptaglycol ether,  
 2 parts N,N-dimethyl-N-hexadecyl-N-(2-oxy-3-sulpho)-propyl-betaine,  
 4 parts benzyl alcohol,  
 200 parts water and  
 756 parts perchloroethylene  
 with a liquor absorption of 104%, and, without inter-

2 parts N,N-dimethyl-N-hexadecyl-N-(2-oxy-3-sulpho)-propyl-betaine,

1 part glacial acetic acid,  
100 parts water and  
857 parts perchloroethylene

15 with a liquor absorption of 100%, dried and steamed at 103°C for 20 minutes.

The fabric is subsequently rinsed in perchloroethylene at 40°C for 3 minutes and freed from the adhering solvent by blowing with air. A clear brilliant yellow dyeing is obtained without the occurrence of waste water.

#### EXAMPLE 4

25 A polyacrylonitrile rope is impregnated with a padding liquor consisting of  
20 parts of a dyestuff preparation consisting of  
34 parts of the dyestuff of the formula



mediate drying, steamed with steam at 103°C for 15 minutes.

The fabric is subsequently rinsed with a solution at 60°C of

2 parts of a mixture consisting of  
24.6 parts N,N-dimethyl-N,N-bis-octadecyl ammonium chloride  
17.5 parts oleic acid heptaglycol ether  
57.9 parts of water in  
1600 parts perchloroethylene.

After drying, an intense red dyeing is obtained without the occurrence of waste water.

### EXAMPLE 3

A polyacrylonitrile fabric is padded on a foulard with a thickened padding liquor consisting of

30 parts of a dyestuff preparation consisting of  
17.3 parts of the dyestuff salt of the formula

8 parts water  
32 parts benzyl alcohol and  
26 parts isopropanol  
1 part glacial acetic acid

40 parts of a stock emulsion consisting of:

1 part oleic acid ethanolamide,  
1 part oleylalcohol eicosaglycol ether,  
4 parts water and  
6 parts perchloroethylene.

as well as 939 parts perchloroethylene

as well as 959 parts perchloroethylene with a liquor absorption of 100% and, without intermediate drying, steamed at 103°C for 10 minutes. To remove the non-fixed dyestuff, the rope is rinsed in perchloroethylene at 45°C for 5 minutes and subsequently dried with hot air. A clear greenish yellow dyeing of good fastness properties is obtained without the occurrence of waste water.

### EXAMPLE 5



25 parts butyrolactone and  
 57.7 parts perchloroethylene,  
 3.5 parts glycerol monoacetate,  
 3.5 parts methylglycol acetate,  
 3 parts nonylphenol decaglycol ether

A fabric of anion-modified polyethylene terephthalate fibres is impregnated with a padding liquor consisting of  
65      60 parts of a dyestuff preparation consisting of  
            15.7 parts of the dyestuff of the formula



58.8 parts perchloroethylene and  
 25.5 parts butyrolactone,  
 1 part glacial acetic acid  
 40 parts of a stock emulsion consisting of:  
 1 part oleic acid ethanolamide,  
 1 part oleyl alcohol eicosaglycol ether,  
 4 parts water and  
 6 parts perchloroethylene  
 as well as 899 parts perchloroethylene  
 with a liquor absorption of 104% and, without intermediate drying, steamed at 115°C for 15 minutes. To remove the non-fixed dyestuff, the fabric is rinsed in perchloroethylene at 45°C for 5 minutes. It is subsequently dried with hot air. A clear pink dyeing is obtained without the occurrence of waste water.

### EXAMPLE 6



A fabric of poly- $\epsilon$ -caprolactam is impregnated with a padding liquor consisting of  
10 parts of the dyestuff of the formula



10 32 parts of a stock emulsion consisting of:  
1 part oleyl alcohol heptadecaglycol ether,  
1 part oleic acid ethanolamide,  
4 parts water and  
6 parts perchloroethylene

15 as well as 958 parts perchloroethylene  
with a liquor absorption of 64% and, without intermediate drying, steamed at 105°C for 10 minutes. The fabric is subsequently rinsed in perchloroethylene at 45°C for 5 minutes and then dried with hot air. A clear blue

20 dyeing of good fastness properties is obtained without the occurrence of waste water.

### EXAMPLE 7

A yarn of polyhexamethylene-diamine adipate threads is sprayed in stripes with a dyestuff solution consisting of

11 parts of the system of the formula

and 85 parts diethylene glycol monobutyl ether in 950 parts trichloroethylene dried and steamed at 103°C for 15 minutes. The yarn is subsequently rinsed in trichloroethylene at 45°C for 5 minutes and then dried by blowing with hot air. A clear yellow unlevel dyeing of good fastness properties is obtained without the occurrence of waste water.

**EXAMPLE 8**

Combed material is sprayed with a dyestuff solution consisting of

50 parts of a dyestuff preparation consisting of  
15 parts of the dyestuff of the formula

and 85 parts diethylene glycol monobutyl ether in 950 parts trichloroethylene and, without intermediate drying, steamed at 103°C for 15 minutes. The combed material is subsequently rinsed in trichloroethylene at 45°C for 5 minutes and then dried by blowing with hot air. A clear green un-level dyeing of good fastness properties is obtained.

## EXAMPLE 9

A fabric of poly- $\epsilon$ -caprolactam is impregnated with a padding liquor consisting of



3.0 parts of the fluorescent dyestuff of the formula

1 part oleic acid ethanolamide,  
1 part oleyl alcohol heptadecaglycol ether,  
4 parts water and

991 parts trichloroethylene

with a liquor absorption of 64% and steamed at 105°C for 15 minutes. The fabric is subsequently rinsed in trichloroethylene at room temperature for 4 minutes, then centrifuged and freed from the adhering solvent by blowing with hot air. A strongly and evenly brightened white fabric is obtained without the occurrence of waste water.

We claim:

1. Pad steaming process for the continuous dyeing and printing of fiber material containing ionic groups comprising the steps of

A. impregnating said fiber material which is selected from the group consisting of natural polyamides, synthetic polyamides, anionically modified synthetic polyamides, anionically modified polyacrylonitrile and anionically modified polyesters with pad-liquor consisting essentially of a solution of 1. a salt or addition product of a lipophylic compound and an ionic dyestuff having the opposite charge of the ionic groups on said fiber material; in

2. organic solvent said organic solvent consisting of a chlorinated hydrocarbon solvent having a boil-

ing point between 40°C and 170°C;

3. up to 10% by weight of water based on said chlorinated hydrocarbon solvent; and
4. 0 to 5% by weight based on said chlorinated hydrocarbon solvent of an emulsifier which forms a thickened emulsion in the presence of water and chlorinated hydrocarbon solvent;

B. subjecting the fiber material to a treatment with steam.

10 2. The process of claim 1 in which the fiber material is subjected to an intermediate drying step before the steam treatment step (B).



20 3. The process of claim 1 in which the fiber material is rinsed with chlorinated hydrocarbon solvent to remove non-fixed dyestuff subsequent to the steam treatment step (B).

4. The process of claim 1 in which said fiber material 25 is wool; synthetic polyamide, polyacrylonitrile containing anionic groups selected from sulfonic acid, sulfide, carboxyl and phosphonic acid groups; polyesters with carboxyl or sulfonic acid groups; or polyamide with sulfonic acid groups.

5. The process of claim 1 in which the pad-liquor contains in addition to the amine salt or addition product (1) and the chlorinated hydrocarbon solvent (2); (3) an auxiliary which assists in the fixing of the dyestuff.

6. The process of claim 1 in which the pad-liquor contains in addition to the amine salt or addition product (1) and the chlorinated hydrocarbon solvent (2); (3) an auxiliary which improves the levelness of the dyeing.

7. The process of claim 1 in which the pad-liquor contains in addition to the amine salt or addition product (1) and the chlorinated hydrocarbon solvent (2); (3) 0.1 to 2 percent by weight of a lower carboxylic acid based on the weight of chlorinated hydrocarbon solvent.

8. The fiber material dyed by the process of claim 1.

\* \* \* \* \*